

## UNITED STATES PATENT OFFICE

2,554,373

## PROCESS FOR PRODUCING GLOSSY COATINGS ON BATHWARE AND METAL

Aymon Francois Max-Claudet, Orly, France, assignor to Societe des Usines Chimiques Rhone-Poulenc, Paris, France, a French body corporate

No Drawing. Application June 1, 1948, Serial No. 30,505. In France June 16, 1947

2 Claims. (Cl. 117—23)

1

This invention relates to vitrifiable compositions and to the use of such compositions.

The most fusible vitrifiable mineral compositions at present known, and employed in particular in the ceramic industries, glaze at about 500° C. or, at the very lowest, at about 450° C.

It has now been found, and this forms the basis of the present invention, that compositions obtained by the fusion of boric acid or boric anhydride and of lead oxide in variable proportions can be employed as vitrifiable compositions at much lower temperatures, in the case of the most fusible compositions as low as 280° C.

It is stated in the literature that when such compositions are slowly heated they have "softening points" at temperatures which vary from 280° C. to 480° C., according to the composition. It has now been found, however, that such compositions in fact return to the liquid state at the said temperatures and then, if the action of the temperature is prolonged to even a small extent they become devitrified and rapidly return to the solid crystalline state.

In the present invention, use is made of this phenomenon in order to obtain glossy coatings on supports consisting of metal or the like (glass, ceramics), and according to the present invention, therefore, a process for the production of a glossy coating on a support comprises applying to the support a composition obtained by fusing together boric acid or boric anhydride and lead oxide, heating the composition until it vitrifies and then immediately withdrawing the coated support from the source of heat.

It has also been found that the liquid phase may be stabilised to some extent, i. e. the return to the solid state may be retarded, by adding to the compositions small quantities of third substances. Examples are alkaline phosphates or the oxides of zinc, nickel, cobalt, tin, aluminum or silicon employed, either separately or in combination, in the form of chemically pure products or in the form of natural minerals containing these elements. Feldspar and kaolin are particularly favourable agents for retarding the return to the solid state.

The optimum proportion of such "stabilising" agents lies between 0.5 and 5%, and preferably at about 2%. In fact, the favourable action of the agent increases with the percentage in which it is employed, but beyond a certain value it brings about a rise in the melting point.

The following examples, in which the parts are by weight, serve to illustrate the invention

but are not intended to limit the invention in any way. Although these examples all concern compositions in which boric anhydride and lead oxide are in the ratio of about 1:9, the invention must not be considered as being limited to these particular proportions, which have only been chosen because they give the most fusible compositions.

2

## Example I

There are intimately mixed:

|                     | Parts |
|---------------------|-------|
| Hydrated boric acid | 17.8  |
| Minium              | 92.1  |

These elements are combined by fusion until completely homogeneous, whereafter the mixture is run off and crushed. The product thus prepared is applied to a metal or ceramic support and it is brought to a temperature of about 280-300° C. As soon as the formation of a glossy vitrified coating is observed, the article is rapidly withdrawn from the source of heat. The coating remains glossy when cooled.

## Example II

There are thoroughly mixed:

|                     | Parts |
|---------------------|-------|
| Hydrated boric acid | 17.8  |
| Minium              | 92.1  |
| Cobaltous carbonate | 4     |

This mixture is fused, run off and crushed as in the preceding example. When heated, it gives a glossy black coating as soon as a temperature of 280-300° C. is reached and remains glossy up to 350° C., beyond which devitrification sets in. In contrast, in a mixture containing no cobaltous carbonate the devitrification follows shortly after fusion.

## Example III

There are thoroughly mixed:

|                         | Parts |
|-------------------------|-------|
| Crystallised boric acid | 17.8  |
| Minium                  | 92.1  |
| Tin oxide               | 2     |
| Kaolin                  | 2     |

When fused, run off and crushed as hereinbefore described, such a mixture has a zone of practical stability after fusion which ranges from 300° C. to 400° C. It crystallises at about 400° C. and returns to the stable liquid state at about 450° C., whereas when no stabilising agents are employed the matting consequent upon crystallisation follows shortly after fusion at 300° C.

## 3

## Example IV

|            | Parts |
|------------|-------|
| Boric acid | 17.8  |
| Minium     | 92.1  |
| Tin oxide  | 2     |

When treated as hereinbefore described, the mixture melts at 300° C. and commences to recrystallise at about 350° C. (in the absence of tin oxide, crystallisation follows shortly after fusion at 10 300° C.) It then melts in stable fashion at about 450° C.

## Example V

There are thoroughly mixed:

|                     | Parts |
|---------------------|-------|
| Hydrated boric acid | 17.8  |
| Minium              | 92.1  |
| Kaolin              | 4     |

The ingredients are fused until completely homogeneous and the resulting composition is run off and cooled. The composition is then crushed and applied to a suitable support. Upon heating, it is found that a glossy and stable coating is formed as soon at a temperature of 300° C. is reached, and this coating can be brought to higher temperatures without destroying the gloss of the coating. In contrast, a similar mixture which does not contain any kaolin is devitrified as soon as it is heated to a temperature slightly above 300° C.

The compositions can be coloured or their natural colour may be modified by adding small quantities of normal ceramic colours generally known under the name "colouring oxides."

I claim:

1. Process for the production of glossy coatings

## 4

on supports selected from the class consisting of earthenware and metal supports, which comprises applying to the support a layer of a composition consisting to the extent of at least 95% by weight of a particulate fused mixture of lead oxide and boric oxide substantially in the proportion of 9 parts by weight of the former to 1 part by weight of the latter, heating the composition up to the temperature at which it first vitrifies and then immediately withdrawing the coated support from the source of heat.

2. Process for the production of glossy coatings on supports selected from the class consisting of earthenware and metal supports, which comprises applying to the support a layer of a particulate fused composition consisting to the extent of at least 95% by weight of a mixture of lead oxide and boric oxide and to the extent of 0.5 to 5% by weight of a stabilizing agent containing an oxide selected from the class consisting of the oxides of zinc, nickel, cobalt, tin, aluminum and silicon, the ratio of boric oxide to lead oxide in the composition being of the order of 1:9, heating the support thus coated up to the temperature at which the composition first vitrifies and then immediately withdrawing the coated support from the source of heat.

AYMON FRANÇOIS MAX-CLAUDET.

## REFERENCES CITED

The following references are of record in the file of this patent:

## UNITED STATES PATENTS

| 35 Number | Name        | Date          |
|-----------|-------------|---------------|
| 2,301,741 | Morris      | Nov. 10, 1942 |
| 2,461,878 | Christensen | Feb. 15, 1949 |